

Feb. 7, 1928.

1,658,647

L. B. MILLER

ALTERNATING CURRENT RECTIFIER

Filed April 14, 1927



Fig. 2.



Inventor:  
Levi B. Miller,  
by *Myron S. Ladd*  
His Attorney.

Patented Feb. 7, 1928.

1,658,647

# UNITED STATES PATENT OFFICE.

LEVI B. MILLER, OF LYNN, MASSACHUSETTS, ASSIGNOR TO GENERAL ELECTRIC COMPANY, A CORPORATION OF NEW YORK.

## ALTERNATING-CURRENT RECTIFIER.

Application filed April 14, 1927. Serial No. 183,841.

My invention relates to alternating current rectifiers wherein current is transmitted between different solid materials maintained in juxtaposition with one another, and has for its principal object the provision of an improved dry rectifier which is stable in operation, does not deteriorate rapidly, and does not require preliminary operation or forming to establish the unilaterally conductive junction between the different solid materials.

Various types of apparatus have been utilized in the past to rectify the current transmitted between direct and alternating current circuits. Some of these apparatus comprise sheets or disks of different metals spaced apart by a very thin film of insulating material formed between them by subjecting them to an alternating voltage while they are pressed tightly together. These apparatus, as constructed in the past, have not been altogether satisfactory because they require preliminary operation or forming, because they are unstable and deteriorate rapidly in use, or because a high pressure must be maintained between the materials both during formation of the insulation film and during the normal operation of the rectifier. In accordance with my invention, these objections are minimized or altogether avoided by the provision of a rectifier which comprises layers of silicon carbide and graphite or carbon so joined together as to form a mechanically inseparable mass. Throughout the specification and claims, the expression "carbonaceous material" will be used to designate carbon, graphite and materials having like characteristics. My invention will be better understood from the following description when considered in connection with the accompanying drawing and its scope will be pointed out in the appended claims.

Referring to the drawings, Fig. 1 is a cross-section view of a rectifier constructed in accordance with my invention; and Fig. 2 is a wiring diagram of a rectifying system wherein my invention has been embodied.

The rectifier illustrated by Fig. 1 comprises a bolt 1 provided with nuts 3 and 4 and surrounded by an insulation sleeve 5 upon which are supported a plurality of rectifying elements each comprising a layer 6 of silicon carbide and a layer 7 of graphite, carbon or the like. In order to ensure a

good conductive connection between these rectifying elements, they are spaced apart by disks 8 of lead or other soft metal which is readily pressed into intimate contact with their surfaces by means of the nuts 3 and 4. Connections to the source of current supply are made through a terminal 9 and a terminal 10 which is insulated from the bolt 1 and nut 3 by the insulation sleeve 5 and an insulation washer 11. It has been found that current, considered as flowing from positive to negative, is readily transmitted from the silicon carbide to the graphite but is transmitted with great difficulty in the reverse direction. It should be understood that the particular structure illustrated is only one of the many forms in which my invention may be utilized.

Fig. 2 illustrates a system wherein an alternating current circuit 12 and a direct current device 13, such as a storage battery, are interconnected through a transformer 14, a smoothing reactor 15, and a pair of rectifiers 16 and 17. With these connections, both halves of the alternating current wave are rectified and fluctuation in the rectified current is minimized by the reactor 15.

The rectifying units 6-7 may be produced by subjecting graphite slabs to the vapors formed in a furnace containing fused quartz or other silicious materials such as a mixture of quartz and carbon particles or a mixture of quartz and silicon carbide. By this process, these vapors or their reduction products are brought into contact with a graphite slab and a tightly adhering layer of silicon carbide is formed on the graphite. The thickness of this layer is dependent both on the concentration of the vapors and on the duration of the treatment to which the graphite is subjected and can be varied at will, but should not be made too thick for the reason that it increases the resistance of the rectifying unit. A layer having a thickness of approximately .02 inches has been found satisfactory for ordinary purposes. It should be understood that the carbide coating of the graphite may be produced not only by the vapor emanating from fused quartz but also by the deposition of the carbide itself from the vapor state or by the vapors emanating from heated carbides, oxy-carbides and the like.

The embodiment of the invention illustrated and described herein has been selected

for the purpose of clearly setting forth the principles involved. It will be apparent, however, that the invention is susceptible of being modified to meet the different conditions encountered in its use and I therefore aim to cover by the appended claims all modifications within the true spirit and scope of the invention.

What I claim as new and desire to secure by Letters Patent of the United States, is,—

- 5 1. An alternating current rectifier comprising a layer of graphite, and a layer of a carbide mechanically united with said layer of graphite.

2. An alternating current rectifier comprising a layer of graphite, and a layer of silicon carbide.

3. An alternating current rectifier comprising a layer of a carbonaceous material, and a layer of a carbide mechanically united 20 with said layer of carbonaceous material.

4. An alternating current rectifier provided with an integral unit comprising a layer of graphite and a layer of silicon carbide.

In witness whereof, I have hereunto set my hand this 12th day of April, 1927.

LEVI B. MILLER.